

# United States Patent [19]

Graf

[11] 3,853,494

[45] Dec. 10, 1974

## [54] CARD CLOTHING

75/123 J, 123 N

[75] Inventor: Werner Graf, Freienbach,  
Switzerland

[73] Assignee: Graf & Cie. A.G., Rapperswil,  
Switzerland

[22] Filed: May 8, 1972

[21] Appl. No.: 252,516

## [30] Foreign Application Priority Data

May 12, 1971 Switzerland..... 7037/71

[52] U.S. Cl..... 29/193.5, 19/114, 75/123 J,  
75/123 N, 75/123 J;123 N

[51] Int. Cl..... B21f 45/10

[58] Field of Search..... 19/114; 29/193.5;

[56]

## References Cited

### UNITED STATES PATENTS

|           |         |                  |          |
|-----------|---------|------------------|----------|
| 1,643,054 | 9/1927  | Brown.....       | 75/123 J |
| 1,707,738 | 4/1929  | Mowat et al..... | 19/114   |
| 1,959,398 | 5/1934  | Whiteley .....   | 75/123 J |
| 2,002,079 | 5/1935  | Dickie.....      | 19/114   |
| 3,151,362 | 10/1964 | Freitag.....     | 19/114   |

Primary Examiner—Winston A. Douglas

Assistant Examiner—O. F. Crutchfield

Attorney, Agent, or Firm—Edward J. Brenner

[57]

## ABSTRACT

Card clothing formed of alloyed steel.

11 Claims, No Drawings

1  
CARD CLOTHING

BACKGROUND OF THE INVENTION

The present invention relates to improvements in card clothing.

Such clothing is especially employed as sawtooth covers for card cylinders. They serve to process fiber material and thus come into engagement with counter elements.

Previously such card clothing was formed of non-alloyed steel and attempts to achieve the desired hardness were made by varying the carbon content of the steel. Yet a certain hardness could not be exceeded since otherwise the material becomes brittle.

SUMMARY OF THE INVENTION

Hence it is a primary object of the present invention to provide card clothing having increased longevity of use and which can be operated at greater speeds than heretofore possible.

Now in order to implement the aforementioned object and others which will become more readily apparent as the description proceeds the card clothing of the present invention is formed of alloyed steel.

DETAILED DESCRIPTION OF THE INVENTION

As explained above an essential aspect of this development resides in forming the clothing from an alloyed steel. It has been found that in contrast to prior attempts at influencing the hardness of the clothing through the carbon content, it is possible to obtain higher hardness values, up to 1,200 Vicker's hardness, with alloyed steels and with increased tensile strength of the material.

Clothing formed in the manner taught by the invention possesses increased longevity and, in other words, with average good nep values can process up to 500 tons staple fiber material formed of natural fibers as well as fibers formed of natural and synthetic polymers. A further advantage which can be realized with the present invention resides in the drastic reduction in the grinding required during the life of the card clothing. It is possible to considerably increase the intervals between the grinding operations owing to the increased service life of the clothing.

In consideration of the previously discussed properties of the card clothing of this invention it is possible to employ advantageously clothing formed completely of alloyed steel at high output cards.

Particularly suitable as the alloys are those containing 0.3 to 2.0 % by weight carbon, 0.05 to 2.25 % by weight silicon, 0.05 to 2.0 % by weight manganese, 0.01 to 2.0 % by weight vanadium, with the remainder iron.

The vanadium can be replaced by 0.01 to 3.5 % by weight tungsten.

The aforementioned alloys can also contain both vanadium and tungsten in the indicated amounts and, if desired, additionally can contain 0.001 to 3.0 % by weight boron.

It is also possible that the aforementioned alloys further contain 0.05 to 4.5 % by weight chromium or titanium.

Similarly it has been found to be advantageous if there is added to one of the previously indicated combi-

nation of components 0.05 to 3.5 % by weight nickel.

A particularly advantageous alloy contains, for instance, 0.5 to 0.6 % by weight carbon, 0.5 to 0.8 % by weight manganese, 1.2 to 1.6 % by weight silicon, and 0.5 to 0.8 % by weight chromium.

On the average there can be realized with the indicated alloys hardness values, based on a Vicker's diamond pyramid hardness test, of approximately 980 with increased toughness of the material, so that card clothing formed of such materials exhibit increased longevity and simultaneously increased card efficiency.

The clothing disclosed herein can be particularly advantageously employed for carding at carding machines. The clothing contains one or a number of wire-shaped structures having a sawtooth profile, the wire-shaped structures consisting of one of the aforementioned alloys.

Of course, the previously disclosed alloys contain the usual amounts of traces of phosphorous and sulphur.

While there is shown and described present preferred embodiments of the invention, it is to be distinctly understood that the invention is not limited thereto but may be otherwise variously embodied and practiced within the scope of the following claims.

Accordingly, what is claimed is:

1. A card clothing containing at least one wire-shaped structure having a sawtooth profile formed of alloyed steel wherein the alloy contains 0.3 to 2.0 percent by weight carbon, 0.05 to 2.5 percent by weight silicon, 0.05 to 2.0 percent by weight manganese and 0.01 to 2.0 percent by weight vanadium, said alloyed steel having a hardness substantially higher than that of the corresponding non-alloyed steel and up to about 1,200 based on the Vickers hardness test.

2. The card clothing as defined in claim 1, wherein the alloy further contains 0.01 to 3.5 percent by weight tungsten.

3. The card clothing as defined in claim 1, wherein the alloy further contains 0.05 to 4.5 percent by weight chromium.

4. The card clothing as defined in claim 1, wherein the alloy contains 0.001 to 3.0 percent by weight boron.

5. The card clothing as defined in claim 1, wherein the alloy contains 0.05 to 3.5 percent by weight nickel.

6. The card clothing as defined in claim 1, wherein the alloy contains titanium.

7. A card clothing containing at least one wire-shaped structure having a sawtooth profile formed of alloyed steel wherein the alloy contains 0.3 to 2.0 percent by weight carbon, 0.05 to 2.5 percent by weight silicon, 0.05 to 2.0 percent by weight manganese and 0.01 to 3.5 percent by weight tungsten, said alloyed steel having a hardness substantially higher than that of the corresponding non-alloyed steel and up to about 1200 based on the Vickers hardness test.

8. The card clothing as defined in claim 7, wherein the alloy contains 0.001 to 3.0 percent by weight boron.

9. The card clothing as defined in claim 7, wherein the alloy contains 0.05 to 3.5 percent by weight nickel.

10. The card clothing as defined in claim 7, wherein the alloy contains titanium.

11. The card clothing as defined in claim 7, wherein the alloy contains 0.05 to 4.5 percent by weight chromium.